

No. 857,927.

PATENTED JUNE 25, 1907.

H. H. DOW, W. S. GATES & A. E. SCHAEFER.

PROCESS OF RECOVERING THE NICKEL CONTAINED IN BASIC NICKEL  
PRECIPITATES.

APPLICATION FILED APR. 18, 1906.



Witnesses,

*G. M. Gaywell*  
John T. Oberlin

Inventors,

Herbert H. Dow, Walter S. Gates,  
and Arthur E. Schaefer,  
By *J. B. Fay*  
their attorney.

# UNITED STATES PATENT OFFICE.

HERBERT H. DOW AND WALTER S. GATES, OF MIDLAND, MICHIGAN,  
AND ARTHUR E. SCHAEFER, OF CLEVELAND, OHIO, ASSIGNEES,  
BY MESNE ASSIGNMENTS, TO THE ONTARIO NICKEL COMPANY, LTD.,  
OF WORTHINGTON, CANADA, A CORPORATION OF CANADA.

## PROCESS OF RECOVERING THE NICKEL CONTAINED IN BASIC NICKEL PRECIPITATES.

No. 857,927.

Specification of Letters Patent.

Patented June 25, 1907.

Application filed April 18, 1906. Serial No. 312,501.

*To all whom it may concern:*

Be it known that we, HERBERT H. Dow and WALTER S. GATES, of Midland, county of Midland, Michigan, and ARTHUR E. SCHAEFER, of Cleveland, county of Cuyahoga, Ohio, citizens of the United States, have invented a new and useful Improvement in Processes of Recovering the Nickel Contained in Basic Nickel Precipitates, of which the following is a specification, the principle of the invention being herein explained, and the best mode in which we have contemplated applying that principle, so as to distinguish it from other inventions.

Our invention relates to methods of rendering soluble the nickel contained in basic nickel precipitates when the latter are treated with free halogens, for instance, when nickelous hydrate or nickelous carbonate, as  $\text{NiCO}_3 \cdot \text{NiO}_2 \text{H}_2$  or a mixture of the two is to be dissolved and perhaps later electrolyzed for metallic nickel.

Said invention consists of steps hereinafter fully described and specifically set forth in the claims.

The annexed description sets forth in detail certain steps embodying the invention, such disclosed steps constituting but one of various ways in which the principle of the invention may be used.

An approved form of apparatus for carrying out the steps thus described is conventionally illustrated in the single figure of the annexed drawing.

It is well known that when basic nickel precipitates, such as the hydrate and the carbonate, are treated with free halogens, such as chlorin and bromin, only a part of the nickel is dissolved to soluble haloids, and the balance remains insoluble, having been oxidized by the halogen to black nickelic hydrate, which latter remains insoluble unless it be dissolved in acid, or unless a very strong halogen be used, in which latter case some of the nickelic hydrate ( $\text{NiO}_3 \text{H}_3$ ) may be dissolved, giving a dark-colored unstable solution, which readily decomposes upon stand-

ing or heating, thus giving off the halogen and reprecipitating the black nickelic hydrate. The action of the halogen upon the nickel 50 hydrate is as follows:



by which it will be noted that only one-third of the nickel has been rendered soluble. The 55 proportion of nickel which is rendered soluble varies according to circumstances, but the ratio of the soluble nickel to the insoluble can never exceed the ratio of one to two, by which it will be noted that no more than one-third 60 of the nickel can be dissolved with dilute halogens. A given amount of chlorin which acts for a length of time great enough to give complete action, would produce 33½% of soluble nickel. We have found that the 65 strength of the halogen has no influence on the above ratio in so far as ultimate results are concerned, but a strong halogen will, of course, act more rapidly. It will be evident, therefore, that in order to dissolve all of the 70 nickel by means of the halogen, it will be necessary to have some reducing agent present which will prevent the formation of nickelic hydrate. Such reducing agents which might be used are carbon compounds, such as oils, 75 etc., any of which would, however, introduce soluble carbon compounds into the solution, which would be undesirable for electrolytic purposes; but we have discovered that the element sulfur in some form, either alone, or in some sulfur-containing compound such as 80 hydrogen sulfid, sulfur dioxid or sulfur chlorid, the latter either  $\text{S}\text{Cl}_2$  or  $\text{S}_2\text{Cl}_2$ , may be used for this purpose, the sulfur as element not only acting well mechanically, but possessing an immense reducing power in a small 85 bulk and small weight, and at a small expense; having, for instance, three times the reducing power of sulfur in the condition of sulfur dioxid, as

90



and



The reaction when the basic nickel precipitate is treated with free halogen in the presence of sulfur, is as follows:



by which it will be noted that 32 parts by weight of sulfur are sufficient to cause the complete solution of 235 parts by weight of nickel, or 371 parts by weight of nickelous hydrate ( $\text{NiO}_2\text{H}_2$ ). In order to get this action quickly it is necessary to have the sulfur in a very fine state of subdivision, such as ground flowers of sulfur or brimstone, or milk of sulfur, or precipitated sulfur; or sulfur which has been acted upon by halogens previously to the action on the nickel precipitate, for instance, sulfur chlorid ( $\text{S}\text{Cl}_2$ ) the reaction in the latter case being:



In the case where sulfur and nickelous hydrate and chlorin are all present, the action is the same as in the case where sulfur chlorid is made separately and added to a nickel precipitate being treated with a halogen, viz., the chlorin acts upon the sulfur first forming sulfur chlorid, which immediately decomposes in the presence of water as follows:



and these products, upon the addition of more  $\text{Cl}_2$ , produce more  $\text{S}\text{Cl}_2$  from the precipitated sulfur, and  $\text{H}_2\text{SO}_4$  from the  $\text{H}_2\text{S}_2\text{O}_3$ , since



and the latter oxidized by



If  $\text{S}_2\text{Cl}_2$  were used, instead of  $\text{S}\text{Cl}_2$ , as noted above, the products upon decomposition with water are:



which, upon the addition of more chlorin, would give  $\text{S}\text{Cl}_2$  and  $\text{H}_2\text{SO}_4$ , the sulfur producing the  $\text{S}\text{Cl}_2$  and the other sulfur products giving the  $\text{H}_2\text{SO}_4$ , the  $\text{HCl}$  remaining. The sulfur that is precipitated by this decomposition is in an extremely finely divided state, so that it is readily acted upon by the chlorin later.

In the case where sulfur chlorid is made separately and added to a nickel hydrate which is being treated with free halogen, the action is the decomposition of  $\text{S}\text{Cl}_2$ , and the subsequent action of the  $\text{S}\text{Cl}_2$  products upon the nickel hydrate and upon the products of the action of  $\text{Cl}_2$  on the nickel hydrate.

When sulfur is used in the form of  $\text{H}_2\text{S}$  it is evident that the sulfur has a stronger reducing power than it has when used as sulfur alone, since one atom of sulfur in  $\text{H}_2\text{S}$  needs four atoms of oxygen to oxidize it to the  $\text{SO}_3$  condition where only three atoms are neces-

sary for one atom of sulfur when sulfur is used alone. Sulfur alone, if in a finely divided state, will give a complete reaction with strong chlorin in a short time, effecting a solution of 100% of the nickel, and precipitating at no time the black nickellic hydrate; with weak chlorin much more time is required, particularly if it is necessary to use up completely a particular batch of chlorin without replenishing the same. Sulfur chlorid will also give 100% soluble nickel and will effect this result much more rapidly than will sulfur alone.  $\text{S}\text{Cl}_2$  works better than  $\text{S}_2\text{Cl}_2$ . When  $\text{S}\text{Cl}_2$  is utilized, only the theoretical amount need be provided in order to get complete reaction, whereas an excess of sulfur alone must be present in order to get 100% nickel, inasmuch as its physical condition is less favorable to the reaction than is that of  $\text{S}\text{Cl}_2$ . If any of the black nickellic hydrate is once created, it is reduced and dissolved by the sulfur in any of the forms given above when treated with the free halogen, the sulfur as a reducing agent acting as follows: The sulfur, upon being oxidized by  $\text{Cl}_2$ , produces  $\text{HCl} + \text{H}_2\text{SO}_4$ , which dissolves either the nickelous hydrate or the nickellic hydrate as fast as the latter tends to form, the  $\text{SO}_2$  and  $\text{H}_2\text{S}_2\text{O}_3$  formed at the same time keeping the solution reduced by reason of the  $\text{H}_2\text{S}_2\text{O}_3$  going to  $\text{SO}_2$  and the latter effecting the reduction. The excess of chlorin will not affect the solution after the nickel has been reduced and dissolved. In case the basic nickelous precipitate is carbonate, as  $\text{NiCO}_3 \cdot \text{NiO}_2\text{H}_2$ , the reaction is precisely the same, as regards the essentials, for instance,



It will be noted that the soluble nickel obtained by the above described steps is a mixture of chlorids and sulfates, and since the latter are injurious to carbon electrodes they must be removed if the solution is to be utilized for the electrolytic deposition of metallic nickel in a cell with carbon electrodes. This can be accomplished in two ways: (1) by the addition of the proper proportion of  $\text{CaO}_2\text{H}_2$  when the halogen is acting upon the nickel precipitate in the presence of sulfur. By this means the sulfur is removed from the solution as the nearly insoluble gypsum ( $\text{CaSO}_4$ ), and in the usual reaction one molecule of the nickelous hydrate is replaced by one molecule of the calcium hydrate, and one molecule of the nickel sulfate by one molecule of the calcium sulfate:



the system thus remaining constant in bromid, since the method employed does not introduce any bromid from an outside source, there being continually dissolved as

much nickel in the dissolving apparatus as there is plated out in the cell, as will be seen by reference to the closed system of apparatus hereinafter described. Calcium hydrate 5 is typical of any compound of calcium which will be converted to a calcium haloid by the action of chlorin, or sulfur and chlorin, since the calcium hydrate with chlorin forms either calcium hypochlorite or a mixture of calcium chlorid and  $\text{Ca}(\text{ClO})_2$ , with a subsequent reduction of these compounds by means of sulfur to calcium chlorid. (2) By the addition of the proper amount of calcium chlorid or calcium bromid, this  $\text{CaCl}_2$  or  $\text{CaBr}_2$ , being 10 added somewhere in the cycle with a consequent precipitation of the sulfate as  $\text{CaSO}_4$ , the reaction being as follows:

$$4\text{NiO}_2\text{H}_2 + \text{CaBr}_2 + \text{S} + 6\text{Br} = 3\text{NiBr}_2 + \text{NiBr} + \text{CaSO}_4 + 4\text{H}_2\text{O}$$

20 the system thus continually increasing in haloids, since halogen is being added in the form of  $\text{CaCl}_2$  or  $\text{CaBr}_2$ , and there is thus dissolved continually in the dissolving apparatus one and one-third times as much nickel as is being plated out in the cell, which means that the system is continually increasing in nickel haloid, and some of the halogen set free in the cell would necessarily have to be 25 used for some other purpose. The gypsum or calcium sulfate which is thus formed by the above reactions is almost entirely insoluble in a normal solution, but the presence of the metal salts renders a considerable part of 30 it soluble, from which part the solution must be freed because, as noted above, of its damaging the anodes and also, because of its producing warty electrolytic nickel, if the solution is supersaturated with respect to the 35 gypsum and, consequently, a part of the latter separates out. In order to thus completely obtain an electrolyte entirely free of sulfate and suitable for electrolysis with carbon anodes, the clear nickel solution is filtered or decanted off from the agitated mixture, thereby removing the precipitated gypsum, and then the solution is evaporated until it attains a syrupy consistency, at which 40 concentration calcium sulfate becomes entirely insoluble. The solution of the nickel salts may be removed by filtration, decantation, or in any other suitable manner. This 45 degree of concentration varies with different solutions, but an average concentration which we have discovered is a specific gravity of 1.41 in nickel chlorid solutions. The nickel solution can then be electrolyzed for the production of metallic nickel and the regeneration of free halogen, which in turn is 50 transferred back from the cell to the dissolving apparatus, where it may act upon more basic nickel precipitate in the presence of fresh sulfur-containing bodies and fresh calcium hydrate, calcium chlorid, etc.

55 We have discovered that some conditions

aid the reaction of the sulfur, halogen and basic nickel precipitate, for instance, heat, strong chlorin, the presence of salt in the solution which makes the chlorin more soluble or retains more chlorin in solution so that the 70 reaction is facilitated, the presence of bromin even in a slight amount, having the sulfur in a finely divided condition, and having an excess of sulfur if sulfur is used alone.

Any suitable apparatus may be utilized for carrying out our improved process. An approved form of apparatus is that shown in the drawing, to which reference has been previously made. As exemplified in such illustrative apparatus, we have found it convenient, in preparing a solution of nickel for electrolysis, to pump the basic precipitate around a tower system comprising two or more towers A in series (thus there are two shown in aforesaid figure), in order that free halogen from 80 the cell, designated by B, shall meet in the first tower basic precipitate or pulp nearly exhausted. The towers are preferably filled with checker-work  $a$ , as shown, whereby the descending mixture of precipitate, or pulp, is 85 exposed over as large a surface as possible to the ascending halogen vapors. The halogen is drawn from the cell B and thence through the series of towers A by means of a suction fan A' connected with the tower farthest removed from the cell, or by equivalent means. To this tower will obviously be fed the fresh supply of pulp, the sulfur and the other necessary reagents, through a suitable feed pipe 90 A<sup>2</sup> therefor provided; and the fluid mixture 95 as it collects in the lower portion of such first tower is raised by means of a pump A<sup>3</sup> and suitable connections a' a<sup>2</sup> to the top of the tower next in order. A similar pump, not shown, serves to transfer the mixture from 100 this tower to the next, or to the electrolytic cell, as the case may be. It will of course be understood that in practice the liquid flow is not wholly progressive, but is preferably caused to circulate a plurality of times 105 through each tower of the series before being advanced to the next. In the cell the nickel is being continually deposited by the current 110 according to the equation



115 This free bromin is removed from the cell, as stated, by the air blast maintained by fan A' and carried to the first tower. In order to produce a good plate the conditions of concentration, temperature, and current density are carefully regulated. The pulp that is being circulated in the towers becomes more fluid as its nickel becomes dissolved, so that 120 more pulp must be added continually, and thus a solution of nickel haloids of any desired strength may be obtained. This solution of nickel haloids is finally cleansed of suspended matter and gypsum and supplied 125 continuously to the cell.

We find it preferable to construct the cell of wood, protected with tar, provided with a water seal, and to use carbon anodes and sheet nickel cathodes.

5. In all the above treatments we have discovered that cobalt acts in the same manner as nickel and in every way is an equivalent of the latter.

Having thus described our invention in detail, that which we particularly point out and distinctly claim is:

1. In a process of rendering soluble the nickel contained in basic nickel precipitates, the step which consists in treating such a precipitate with free halogen in the presence of sulfur.

2. In a process of rendering soluble the nickel contained in basic nickel precipitates, the step which consists in treating such a precipitate with free halogen in the presence of finely-divided sulfur.

3. In a process of rendering soluble the nickel contained in basic nickel precipitates, the step which consists in treating such a precipitate with free halogen in the presence of a sulfur-containing body.

4. In a process of rendering soluble the nickel contained in basic nickel precipitates, the step which consists in treating such a precipitate with free halogen in the presence of a sulfur-containing compound.

5. In a process of rendering soluble the nickel contained in basic nickel precipitates, the step which consists in treating such a precipitate with free halogen in the presence of a sulfur haloid.

6. In a process of rendering soluble the nickel contained in basic nickel precipitates, the step which consists in treating such a precipitate with free halogen in the presence of sulfur chlorid.

7. In a process of rendering soluble the nickel contained in basic nickel precipitates, the step which consists in treating such a precipitate with free bromin in the presence of sulfur.

8. In a process of rendering soluble the nickel contained in basic nickel precipitates, the step which consists in treating such a precipitate with free bromin in the presence of finely-divided sulfur.

9. In a process of rendering soluble the nickel contained in basic nickel precipitates, the step which consists in treating such a precipitate with free bromin in the presence of a sulfur-containing body.

10. In a process of rendering soluble the nickel contained in basic nickel precipitates, the step which consists in treating such a precipitate with free bromin in the presence of a sulfur-containing compound.

11. In a process of rendering soluble the nickel contained in basic nickel precipitates, the step which consists in treating such a pre-

cipitate with free bromin in the presence of 65 a sulfur haloid.

12. In a process of rendering soluble the nickel contained in basic nickel precipitates, the step which consists in treating such a precipitate with free bromin in the presence of 70 sulfur chlorid.

13. In a process of recovering nickel from basic nickel precipitates, the steps which consist in treating such a precipitate with free halogen in the presence of a sulfur-containing 75 body with the formation of nickel haloid; and, then, electrically dissociating such haloid.

14. In a process of recovering nickel from basic nickel precipitates, the steps which consist in treating such a precipitate with free 80 halogen in the presence of a sulfur-containing body with the formation of nickel haloid; electrically dissociating such haloid with the formation of metallic nickel and the liberation of free halogen; and, then, treating 85 a fresh quantity of said precipitate with such liberated halogen.

15. In a process of recovering the nickel contained in basic nickel precipitates, the steps which consist in treating such a precipitate in a dissolving apparatus with free halogen in the presence of a sulfur-containing body with the formation of nickel haloid; electrically dissociating in a cell such haloid with the formation of metallic nickel and the 95 liberation of free halogen; and transferring the latter from the cell back to the dissolving apparatus.

16. In a process of recovering the nickel contained in basic nickel precipitates, the 100 steps which consists in treating such a precipitate in a dissolving apparatus with free halogen in the presence of a sulfur haloid with the formation of nickel haloid; electrically dissociating in a cell such haloid with the 105 formation of metallic nickel and the liberation of free halogen; and transferring the latter from the cell back to the dissolving apparatus.

17. In a process of recovering the nickel 110 contained in basic nickel precipitates, the steps which consist in treating such a precipitate in a dissolving apparatus with free bromin in the presence of finely-divided sulfur with the formation of nickel bromid; 115 electrically dissociating in a cell such bromid with the formation of metallic nickel and the liberation of free bromin; and transferring the latter from the cell back to the dissolving apparatus.

18. In a process of rendering soluble the nickel contained in basic nickel precipitates, the step which consists in treating such a precipitate with free halogen in the presence of a sulfur-containing body and a reagent capable of precipitating the sulfate from nickel sulfate radical.

19. In a process of rendering soluble the

nickel contained in basic nickel precipitates, the step which consists in treating such a precipitate with free halogen in the presence of a sulfur containing body and a reagent capable of precipitating the sulfate radical from nickel sulfate as calcium sulfate.

20. In a process of rendering soluble the nickel contained in basic nickel precipitates, the step which consists in treating such a precipitate with free bromin in the presence of a sulfur-containing body and a soluble calcium salt.

21. In a process of rendering soluble the nickel contained in basic nickel precipitates, the step which consists in treating such a precipitate with free bromin in the presence of a sulfur haloid and calcium hydrate.

22. In a process of rendering soluble the nickel contained in basic nickel precipitates, the steps which consist in treating such a precipitate with free halogen in the presence of sulfur, whereby nickel haloid and sulfate are formed; and, then, precipitating the sulfate radical from such nickel sulfate.

23. In a process of recovering the nickel contained in basic nickel precipitates, the steps which consist in treating such a precipitate with free halogen in the presence of sulfur, whereby nickel haloid and sulfate are formed; removing such sulfate; and, then, electrically dissociating such nickel haloid.

24. In a process of recovering the nickel contained in basic nickel precipitates, the steps which consist in treating such a precipitate with free halogen in the presence of sulfur, whereby nickel haloid and sulfate are formed; precipitating the sulfate from such nickel sulfate; electrically dissociating such nickel haloid with the formation of metallic nickel and the liberation of the halogen; and, then, treating fresh precipitate with such liberated halogen.

25. In a process of recovering the nickel contained in basic nickel precipitates, the step which consists in treating such a precipitate in a dissolving apparatus with free halogen in the presence of a sulfur-containing body and a reagent capable of precipitating the sulfate radical from nickel sulfate; decanting off the solution containing the nickel haloids thus formed; electrically dissociating in a cell such haloids with the formation of metallic nickel and the liberation of free halogen; and transferring the latter from the cell back to the dissolving apparatus.

26. In a process of recovering the nickel contained in basic nickel precipitates, the steps which consist in treating such a precipitate in a dissolving apparatus with free bromin in the presence of finely-divided sulfur and a reagent capable of precipitating the sulfate radical from nickel sulfate as calcium

sulfate; decanting off the solution containing the nickel bromid thus formed; electrically dissociating in a cell such bromid with the formation of metallic nickel and the liberation of free bromin; and transferring the latter from the cell back to the dissolving apparatus.

27. In a process of rendering soluble the nickel contained in basic nickel precipitates, the steps which consist in treating such a precipitate with free halogen in the presence of a sulfur-containing body and a reagent capable of precipitating the sulfate radical from nickel sulfate; decanting off the solution containing the nickel haloid thus formed; and evaporating the same to a consistency necessary to precipitate the last traces of sulfate.

28. In a process of recovering the nickel contained in basic nickel precipitates, the step which consists in treating such precipitate in a dissolving apparatus with free halogen in the presence of a sulfur-containing body and a reagent capable of precipitating the sulfate radical from nickel sulfate; decanting off the solution containing the nickel haloids thus formed; evaporating the same to a consistency necessary to precipitate the last traces of sulfate; electrically dissociating in a cell the nickel haloids with the formation of metallic nickel and the liberation of free halogens and transferring the latter from the cell back to the dissolving apparatus.

29. In a process of recovering the nickel contained in basic nickel precipitates, the steps which consist in treating such precipitate with free halogen in the presence of a sulfur-containing body and a soluble calcium salt; decanting off the solution containing the nickel haloid thus formed; evaporating the same to a consistency sufficient to precipitate the last traces of sulfate; electrically dissociating in a cell the nickel haloids with the formation of metallic nickel and the liberation of the halogens; transferring the latter from the cell back to fresh basic nickel precipitate to attack the same; and adding to the solution more of the sulfur-containing body and the soluble calcium salt.

Signed by HERBERT H. DOW and WALTER S. GATES, this 14 day of April, 1906.

HERBERT H. DOW.  
WALTER S. GATES.

Attested by—

LEO W. LOWE,  
G. L. CAMP.

Signed by ARTHUR E. SCHAEFER, this 4<sup>th</sup> day of April, 1906.

ARTHUR E. SCHAEFER.

Attested by—

JNO. F. OBERLIN,  
G. W. SAYWELL.

Correction in Letters Patent No. 857,927.

It is hereby certified that in Letters Patent No. 857,927, granted June 25, 1907, upon the application of Herbert H. Dow and Walter S. Gates, of Midland, Michigan, and Arthur E. Schaefer, of Cleveland, Ohio, for an improvement in "Processes of Recovering the Nickel Contained in Basic Nickel Precipitates," an error appears in the printed specification requiring correction, as follows: In line 127, page 4, the word "radical" after the word "sulfate" should be stricken out and inserted after the word "sulfate" in line 126, same page; and that the said Letters Patent should be read with this correction therein that the same may conform to the record of the case in the Patent Office.

Signed and sealed this 24th day of September, A. D., 1907.

[SEAL.]

C. C. BILLINGS,  
*Acting Commissioner of Patents.*